

# United States Patent [19]

Kubota et al.

[11] 3,860,699

[45] Jan. 14, 1975

[54] **RESIN COMPOSITION SUITABLE FOR USE IN HAIR DRESSING PREPARATIONS**

[75] Inventors: **Ikuo Kubota, Kawasaki; Masakatsu Mikami, Nara; Isao Konaka, Uzi; Toshihiko Misaki, Kyoto, all of Japan**

[73] Assignee: **Shinonaga Kasei Co., Ltd., Osaka, Japan**

[22] Filed: **Feb. 6, 1973**

[21] Appl. No.: **330,130**

[52] **U.S. Cl. .... 424/47, 424/71**

[51] **Int. Cl. .... A61k 7/10**

[58] **Field of Search** ..... 424/71, 47

[56] **References Cited**

UNITED STATES PATENTS

|           |         |              |        |
|-----------|---------|--------------|--------|
| 3,405,084 | 10/1968 | Bohac et al. | 424/71 |
| 3,577,517 | 5/1971  | Kubot et al. | 424/71 |
| 3,634,368 | 1/1972  | Palmer       | 424/47 |
| 3,692,893 | 9/1972  | Palmer       | 424/71 |

*Primary Examiner*—Sam Rosen

*Attorney, Agent, or Firm*—Ladas, Parry, Von Gehr, Goldsmith & Deschamps

[57] **ABSTRACT**

A resin composition useful in hair dressing preparations which comprises the resin-containing liquid obtained by refluxing the following copolymerizable monomeric ingredients under copolymerizing conditions in a water-soluble organic solvent; (1) 5-89 percent by weight of a diacetone acrylamide, (2) 5-40 percent by weight of at least one ester of an alkanol having 4-18 carbon atoms and an acid selected from a group consisting of acrylic acid and methacrylic acid, (3) 6-35 percent by weight of at least one acid selected from a group consisting of acrylic acid, methacrylic acid and itaconic acid, (4) 0-84 percent by weight of at least one ester of an alkanol having one to three carbon atoms and an acid selected from a group consisting of acrylic acid and methacrylic acid.

**12 Claims, No Drawings**

## RESIN COMPOSITION SUITABLE FOR USE IN HAIR DRESSING PREPARATIONS

### BACKGROUND OF THE INVENTION

The present invention relates to a resin composition which adheres to hair, exhibiting an excellent hair dressing effect even in hot and highly humid environments.

Recent research in hair dressing materials has been directed to development of a resinous material having the following abilities:

1. To retain the initial shape of the locks curled or set over a prolonged period in any environment;
2. To retain curl and/or wave as set even if the hair is combed or brushed without "flaking," — that is, without the hair dressing preparation scaling off from the hair like dandruff;
3. To give to the locks a natural appearance and a "feel" free from stiffness; and
4. To be easily removable from hair by rinsing with warm water or shampooing.

In the conventional hair dressing preparations, shellac, polyvinylpyrrolidone, polyvinyl methyl ether and the like are used as the binding resin. However, these resins have some defects.

Shellac and the related resins are undesirable because they flake, that is, the film formed with these resins is so brittle that it is easily crumbled by combing or brushing, and scales off the hair and deposits like dandruff on the surface of the hair.

Polyvinylpyrrolidone resins are unsatisfactory, too, in that they form a film on hair that is very hard when dried, but readily softens in the presence of moisture, and the difference between the two states is too remarkable. Therefore, the films of these resins easily flake off in the dried state, and easily lose binding power to maintain curls or wave set when the humidity is high.

Use of the polyvinylpyrrolidone resins in which vinyl acetate is copolymerized has been proposed. These copolymers, however, are not quite free from flaking, and the film formed therewith is poor in transparency and therefore give locks an unnatural appearance.

Polyvinyl methyl ether is extremely sticky and therefore this resin can be used only as a plasticizing additive to polyvinyl pyrrolidone.

Resins known to be free from the above-mentioned defects include copolymers of vinyl methyl ether and maleic anhydride; copolymers of vinyl acetate and an ester of crotonic acid, acrylic acid or methacrylic acid; copolymers of vinylpyrrolidone and an acrylic acid ester etc., and by neutralizing the carboxylic groups contained in said copolymers resins giving water-soluble films are provided.

However, these resins do not exhibit satisfactory curl retention. Hair that is curled and/or set by means of a preparation containing one or more of these resins generally retains the curl or set no longer than several hours, and, in a hot and humid environment, that is, in a bathroom or in rainy weather, for instance, retention power is quickly lost.

Accordingly there has been demand for a further improved binding resin for use in hair dressing preparations.

### SUMMARY OF THE INVENTION

The present invention relates to a novel resin composition which has strong adhesive power, and excellent curl retention even in a hot and highly humid environment and is free from flaking.

This invention is based on the discovery that the foregoing desirable properties useful in hair dressing preparations can be achieved by employing a liquid resin

10 composition which comprises a resin-containing liquid obtained by refluxing the following polymerizable monomeric ingredients under copolymerizing conditions in a water-soluble organic solvent: (1) 5 - 89 percent by weight of diacetone acrylamide, (2) 5 - 40 percent by weight of at least an ester of an alkanol having four to 18 carbon atoms and an acid selected from a group consisting of acrylic acid and methacrylic acid, (3) 6 - 35 percent by weight of at least one acid selected from a group consisting of acrylic acid, methacrylic acid and itaconic acid, and (4) 0 - 84 percent by weight of at least one ester of an alkanol having one to three carbon atoms and an acid selected from a group consisting of acrylic acid and methacrylic acid.

More preferably, the resin composition of this invention 25 comprises a resin-containing liquid obtained by polymerization of a copolymerizable monomeric mixture consisting of (1) 10 - 60 percent by weight of diacetone acrylamide, (2) 10 - 30 percent by weight of an ester of an alkanol having four to 18 carbon atoms and an acid selected from a group consisting of acrylic acid and methacrylic acid, (3) 10 - 20 percent by weight of at least one acid selected from a group consisting of acrylic acid, methacrylic acid and itaconic acid, and (4) 20 - 70 percent by weight of an ester of alkanol having one to three carbon atoms and an acid selected from a group consisting of acrylic acid and methacrylic acid.

Further more preferably, the resin composition of this invention comprises a resin containing liquid obtained by polymerization of a copolymerizable monomeric mixture consisting of (1) 20 - 30 percent by weight of diacetone acrylamide, (2) 15 - 30 percent by weight of an ester of an alkanol having four to 18 carbon atoms and an acid selected from a group consisting of acrylic acid and methacrylic acid, (3) 10 - 20 percent by weight of at least one acid selected from a group consisting of acrylic acid, methacrylic acid and itaconic acid, and (4) 30 - 65 percent by weight of an ester of alkanol having one to three carbon atoms and an acid selected from a group consisting of acrylic acid and methacrylic acid.

The resin composition of this invention is especially suitable for use in hair dressing preparations in the form of pressurized packaging or aerosols. The neutralized composition of this invention is soluble in water and most of the water-miscible organic solvents and its solution in such a solvent exhibits a good mutual solubility with the usual pressurized packaging propellents. The neutralized copolymer, that is, the main binder component, contained in the composition of this invention, can be easily removed from hair by washing with warm water or a usual shampoo.

Now the invention is explained in detail with respect to the constituents of the copolymer constituting the main component of the composition of this invention and the reason for the numerical restrictions imposed on the proportions of the constituents.

Diacetone acrylamide, which is referred to as monomer constituent (1), is water-soluble and its homopolymer is a hygroscopic but water-insoluble substance. Diacetone acrylamide has the formula N-(1,1-dimethyl-3-oxobutyl)acrylamide. It is produced by The Lubrizol Corporation, (Cleveland, Ohio). When this constituent makes up less than 5 percent by weight in the copolymer, the resulting copolymer is, as the whole, insufficiently hydrophilic and is poor in affinity to hair, and therefore the hair dressing preparation comprising this copolymer composition is less spreadable in hair. The copolymer containing more than 89 percent by weight of this monomer constituent is improper in that the resulting film is so hard and brittle. Such a large content of this monomer is improper, too, in consideration of the contents of the other necessary constituents, that is, monomer constituent (3) which contributes to improvement in flexibility and washing-out property of the resulting film and monomer constituent (2) which contributes to hardness of the resulting film and compatibility with the propellant gas.

The monomer constituent (2) must constitute at least 5 percent by weight. Otherwise, a pressurized product (aerosol) system containing such a resin composition is unstable in the coexistence with a halogenated hydrocarbon or liquefied petroleum gas propellant. Further, the resulting film has poor flexibility and flakes. On the other hand when the copolymer contains more than 40 percent by weight of this monomer constituent, the copolymer is only slightly soluble in water and is not easily removed by shampooing. Also such a copolymer gives extremely sticky film which collects dust and soils the hair.

The content of monomer constituent (3), that is, acrylic acid, methacrylic acid, itaconic acid or a mixture thereof, is varied in accordance with the contents of the monomers of classes (1), (2) and (4) so as to provide stable pressurized product systems. When the copolymer contains monomer constituent (3) in an amount of less than 6 percent by weight, the resulting film is water-insoluble. Whereas, the copolymer containing more than 35 percent by weight of this comonomer gives film which is excessively hygroscopic and sticky.

The monomer constituent belonging to class (4) is an ester of an alkanol having one to three carbon atoms and acrylic acid or methacrylic acid. This monomer constituent helps to render the film formed of the resulting resin composition flexible and adhesive. This monomer constituent is not an indispensable component in this invention.

In order to obtain the resin composition with which the object of this invention is achieved, the monomer constituents (1) and (3), which contribute to the enhancement of the hydrophilic property of the copolymer, and the monomer constituents (2) and (4), which contribute to the increment in the hydrophobic property thereof, must be combined in a proper proportion. Namely, if the monomer (1) alone is combined with the monomer (2) and (4) or (2) alone, the resulting resin composition lacks water-solubility and thus it is not easily removed from hair by washing. Whereas, when monomer (3) alone is combined with monomer (2) and (4) or (2) alone, if the content of the monomer (3), which is the hydrophilic constituent, is low, the resulting resin composition is difficult to wash out; and if the content of the monomer (3) is high, the resin composi-

tion becomes too sticky because of its hygroscopic property, and cannot hold curls or wave set for long.

Therefore, it is necessary to combine all of the monomer constituents (1), (2), (3) and (4) in a proper proportion so that the films formed on hair by spraying a hair dressing preparation containing the resulting resin composition may have the desirable combination of water-solubility, hardness and adhesion to hair, which properties are not degraded even at elevated temperatures and/or under high humidity.

For the solution polymerization of said monomers, usually a water-soluble aliphatic alcohol having one to four carbon atoms or a mixture of such alcohols is used as the solvent or reaction medium. A water-containing alcohol, such as 95 percent ethyl alcohol, can be used as the solvent. The polymerization is carried out with stirring at the boiling temperature of the used solvent or at a temperature proximate thereto.

It is an additional advantage of this invention that the control of temperature during polymerization can easily be accomplished and homogeneous polymer products are obtained.

In this invention the polymerization can be practiced in the well known manner in which a polymerization catalyst, e.g., peroxides such as benzoyl peroxide, acetyl peroxide, lauroyl peroxide, etc. and azo-compounds such as azo-bis-isobutyronitrile is suitably employed.

The resin-containing composition resulting from the solution polymerization of the mixture of said monomers is usually neutralized by the addition of a water-soluble basic substance so as to produce the water-soluble resin composition of this invention. Examples of such basic substances are ammonia water, lithium hydroxide, sodium hydroxide, potassium hydroxide, mono-, di-, or tripropanolamine, ammonium salts of lysine or glycine, amino methyl propanol, amino methyl propanediol, and the mixtures thereof, etc.

Since an organic amine compound gives a water-free composition, such an amine compound is preferably used when the resin composition is intended to be used in pressurized package (aerosols) systems where existence of water is generally deleterious.

In another embodiment of this invention the resin composition may additionally contain various additives, such as glycerine, ethylene glycol, sorbitol, polyethylene glycol, lanoline, or dimethyl phthalate for modifying the hardness of the resulting film.

The liquid resin composition for hair dressing preparations obtained by the present invention can be packed in a sealed vessel with or without being dissolved in an water soluble organic solvent, such as an alkanol having one to four carbon atoms, dioxane, methyl ethyl ketone, acetone, ethyleneglycol mono-methyl ether, ethyleneglycol monoethyl ether, etc., pressurized with a propellant as pressurized package products. The propellents to be used in such a case includes halogenated hydrocarbons mainly composed of dichlorodifluoroethane, trichloromonofluoromethane, and/or dichlorotetrafluoroethane; liquefied petroleum gases mainly composed of propane and butane; dimethyl ether, carbon dioxide, or mixtures thereof, which are conventionally used.

Excellent pressurized (aerosol) hair dressing preparations (hair lacquers) can be provided by employing the resin composition of the present invention. That is, the composition is dissolved in an water-soluble organic solvent in a proportion that its solid content is 0.5

– 10 percent by weight of the mixture, and then 25 – 75 percent by weight of the thus formed mixture and 75 – 25 percent by weight of any of the above-mentioned propellents are packed in a sealed vessel.

Further, the resin composition of this invention, which is soluble in water and an water-soluble organic solvent can be used as an ingredient for non-pressurized hair dressing and other cosmetic preparations, such as hair cream, hair lotion, or shaving cream, with addition of the other hair dressing materials. It is also possible to use the resin composition of the invention atomizing by means of an ejector unit such as disclosed in British Pat. Nos. 1,148,484 and 1,172,274.

In still another embodiment of this invention, the resin composition can be used as a film-forming ingredient for beauty packs and as a coating preparation for protecting wounds in the skin.

The invention is best illustrated by the following examples, which are given merely for the exemplary purpose. It is not intended that these examples limit the scope of the invention or the manner in which the present invention can be practiced.

#### DESCRIPTION OF PREFERRED EMBODIMENTS:

##### Example 1

Into a four-necked flask equipped with a reflux condenser, a dropping funnel, a thermometer and an agitator, 250 g of methyl acrylate, 300 g of methyl methacrylate, 150 g of lauryl (dodecyl) methacrylate, 200 g of diacetone acrylamide, 40 g of acrylic acid, 50 g of methacrylic acid, 10 g of itaconic acid, and 500 g of ethyl alcohol were placed and 3 g of benzoyl peroxide was added thereto. The mixture was refluxed for polymerization by heating at 80° – 82°C on a hot bath with constant agitation. After 3 hours further 3 g of benzoyl peroxide dispersed in 50 g of ethyl alcohol was added and heating was continued. After 1.5 hours, a solution of the copolymer in ethyl alcohol was obtained whereby the conversion was 98.5 percent. Then, a solution of 96.3 g of aminomethyl propanediol and 200 g of ethyl alcohol were added to the solution of the copolymer through the dropping funnel and additionally 350 g of ethyl alcohol was supplied, whereby a resin composition containing 50 percent of the nonvolatiles was obtained. The viscosity of this product composition at 20°C was about 27,000 centipoises. The conversion was calculated by measuring the amount of the non-volatile materials therein and the viscosity was measured by a Brookfield type viscometer.

Ten grams (10g) of the thus obtained composition was dissolved in 90 g of ethyl alcohol, and then a perfume was added to the mixture. This mixture was placed in an aerosol container and packed with 150 g of a mixture of equal amounts of trichloromonofluoromethane and dichlorodifluoromethane (1:1 by weight) according to the conventional pressurized packaging technique so as to make a hair lacquer product.

##### Example 2

Into the same four-necked flask as used in Example 1, 140 g of ethyl acrylate, 150 g of ethyl methacrylate, 300 g of stearyl (octadecyl) acrylate, 250 g of diacetone acrylamide, 65 g of acrylic acid, 75 g of methacrylic acid, 20 g of itaconic acid, 200 g of ethyl alcohol, and 300 g of isopropyl alcohol were placed and 3.5 g of azo-bis-isobutyronitrile was added thereto. The

mixture was refluxed for polymerization by heating at 88° – 90°C for 3.5 hours. Thereafter further 1.5 g of azo-bis-isobutyronitrile dispersed in 50 g of ethyl alcohol was added and heating was continued. After 1 hour, a solution of a copolymer in ethyl alcohol was obtained at a conversion of 99 percent. Then a solution of 278.86 g of triisopropanolamine in 300 g of isopropyl alcohol was added to the solution of the copolymer and additionally 420 g of ethyl alcohol was supplied whereby a resin composition containing 50 percent of nonvolatile materials was obtained. The viscosity of this product composition at 20°C was about 15,000 centipoises.

Ten grams (10g) of the thus obtained composition was diluted with 90 g of ethyl alcohol, and then a perfume was added to the mixture. This mixture was placed in an aerosol container and was packed with 150 g of a liquefied gas comprising trichloromonofluoromethane and dichlorodifluoromethane (1:1 by weight) according to the conventional pressurized packaging technique.

##### Example 3

The following copolymerization was carried out in accordance with the procedure of Example 1. Three hundred and fifty grams (350g) of methyl acrylate, 50 g of butyl acrylate, 25 g of butyl methacrylate, 175 g of stearyl (octadecyl) methacrylate, 250 g of diacetone acrylamide, 65 g of acrylic acid, 75 g of methacrylic acid, and 20 g of itaconic acid were mixed with 500 g of ethyl alcohol. To this mixture, 12 g of benzoyl peroxide was added and the whole mixture was heated at 78° – 80°C for polymerization. After 3 hours, further 2 g of benzoyl peroxide dissolved in 20 g of ethyl alcohol was added twice with an interval of 30 minutes. Thus a copolymer was formed at the conversion of 99.5 percent. The thus obtained resin-containing liquid was neutralized by adding 167.67 g of aminomethyl propanediol dissolved in 200 g of ethyl alcohol. The neutralized liquid was further diluted by adding 407 g of ethyl alcohol so that the non-volatile content thereof became about 50 percent by weight.

The viscosity of the thus obtained resin composition was 32,000 cps (measured by a Brookfield viscometer).

Ten grams (10g) of the thus obtained composition was dissolved in 90 g of ethyl alcohol, and a perfume was added to the mixture. This mixture was placed in an aerosol container and packed with 150 g of a mixture of trichloromonofluoromethane and dichlorodifluoromethane (1:1 by weight) according to the conventional pressurized packaging technique so as to make a hair lacquer product.

Also a set lotion was prepared by dissolving 20 g of the thus obtained resin composition (solution) in 56 g of ethyl alcohol and 24 g of water and adding 0.2 g of a perfume. This set lotion was placed in an spray bottle with a manually operated spray pump and used for evaluation. This set lotion exhibited a good curl retention without flaking.

##### Examples 4 – 10

In the same way as in Example 1 – 3, copolymers were prepared, the proportions of the monomer constituents of which are shown in the following Table 1.

Aerosol hair lacquers were prepared using each of the obtained resin compositions in the same way as in Examples 1 - 3.

The performance of the hair lacquers prepared in all these examples was examined by the curl retention test, which evaluates moisture resistance of the formed membrane, the solubility test, which evaluates wash-out property of the membrane, the test for compatibility with aerosol propellents and the Sword Rocker hardness test and the flaking resistance test.

The curl retention was calculated in accordance with the following equation:

$$\text{Curl retention (percent)} = (L - L_t) / (L - L_0) \times 100$$

whereby

$L$ : length of a straight specimen (a bundle of hair).

$L_t$ : length of a curled specimen prior to the test.

$L_0$ : length of a curled specimen after subjected to humid condition for a predetermined period of time.

The test conditions were as follows: For the resin compositions of Examples 1 to 3, the temperature range was 38° - 40°C and RH was 95 percent. For the resin compositions of all the other examples, the temperature was 30°C and RH was 90 percent, and test samples were kept for 10 hours under the humid condition. Greater curl retention values (percent) represent better curl retention, that is, better moisture resistance, and 100% curl retention means perfect retention.

Curl retention of 80 percent or more after 10 hours under the humidity 90 - 95 percent was rated as "ex-

cellent." Curl retention of 65 percent or more was rated as "good." Curl retention of 50 percent or more was rated as "allowable." Curl retention less than 50 percent was rated as "poor."

The solubility or the wash-out property of the resin composition was evaluated by measuring the time required for a membrane 10 mm × 10 mm in area and 0.1 mm in thickness formed with the prepared resin composition to dissolve in water at 20°C. Dissolution time 60 seconds or less was rated as "excellent." Ninety seconds or less was rated as "good," 120 seconds or less as "allowable" and more than 120 seconds as "poor."

The compatibility in the aerosol formulation was determined by measuring the amount of dichlorodifluoromethane that can be homogeneously mixed with 10g of an ethanol solution containing 5 percent by weight of the prepared copolymer at 20°C. Twenty-five grams or more was rated as "excellent," 20 g or more as "good," 15 g or more as "allowable" and less than 15 g as "poor."

The hardness of the formed membrane was tested by means of the Sword Rocker hardness tester. Sword Rocker value 50 or more was rated as "excellent." 40 or more was rated as "good," 30 or more as "allowable" and less than 30 as "poor."

The flaking resistance was evaluated by combing and brushing a bundle of hair on which the hair lacquer had been sprayed and dried, and subjectively rated as "excellent," "good," "allowable" and "poor."

The results of the evaluation tests are summarized in Table 1.

Table 1

| Ex. | Monomer(1) | Monomer(2) | Monomer(3)                | Monomer(4)            | Curl retention | Wash-out property | Compatibility in aerosol formulation | Hardness of coating membrane | Flaking   |
|-----|------------|------------|---------------------------|-----------------------|----------------|-------------------|--------------------------------------|------------------------------|-----------|
|     | (%)        | (%)        | (%)                       | (%)                   |                |                   |                                      |                              |           |
| 1.  | DAA 20     | LMA 15     | AA 4<br>MAA 5<br>IA 1     | 10<br>MMA30           | 55             | excellent         | excellent                            | good                         | excellent |
| 2.  | DAA 25     | SA 30      | AA 6.5<br>MAA 7.5<br>IA 2 | 16<br>EMA15           | 29             | excellent         | good                                 | excellent                    | good      |
| 3.  | DAA 25     | SMA 17.5   | AA 6.5<br>MAA 7.5<br>IA 2 | 16<br>BA 5<br>BMA 2.5 | 42.5           | good              | excellent                            | good                         | excellent |
| 4.  | DAA 10     | EHMA 30    | AA 3<br>MAA 5<br>IA 2     | 10<br>EMA30           | 50             | excellent         | allowable                            | excellent                    | good      |
| 5.  | DAA 10     | SA 10      | AA 3.5<br>MAA 3.5<br>IA 3 | 10<br>EMA35           | 70             | good              | allowable                            | allowable                    | good      |
| 6.  | DAA 60     | SA 10      | AA 8<br>MAA 6<br>IA 6     | 20<br>EA              | 10             | allowable         | excellent                            | allowable                    | allowable |
| 7.  | DAA 60     | SA 30      | AA 3<br>MAA 5<br>IA 2     | 10<br>-               | 0              | good              | good                                 | excellent                    | allowable |
| 8.  | DAA 4      | LMA 20     | AA 5<br>MAA10<br>IA 5     | 20<br>EA 56           | 56             | poor              | excellent                            | good                         | allowable |
| 9.  | DAA 20     | LMA 20     | AA 5<br>MAA10<br>IA 5     | 20<br>EA 40           | 40             | good              | good                                 | excellent                    | excellent |
| 10. | DAA 90     | LMA 4      | AA 2<br>MAA 3<br>IA 1     | 6<br>-                | 0              | good              | good                                 | good                         | excellent |
| 11. | DAA 20     | LMA 4      | AA 5<br>MAA10<br>IA 5     | 20<br>EA 56           | 56             | excellent         | excellent                            | poor                         | poor      |
| 12. | DAA 20     | LMA 41     | AA 5<br>MAA10<br>IA 5     | 20<br>EA 19           | 19             | excellent         | poor                                 | excellent                    | excellent |

Table 1 - Continued

| Ex. Monomer(1) | Monomer(2) | Monomer(3)               | Monomer(4) | Curl retention | Wash-out property | Compatibility in aerosol formulation | Hardness of coating membrane | Flaking                  |
|----------------|------------|--------------------------|------------|----------------|-------------------|--------------------------------------|------------------------------|--------------------------|
| (%)            | (%)        | (%)                      | (%)        |                |                   |                                      |                              |                          |
| 13. DAA 20     | LMA 20     | AA 2<br>MAA 2<br>IA 1    | 5          | EA 55          | 55                | excellent                            | poor                         | excellent good excellent |
| 14. DAA 20     | LMA 20     | AA 11<br>MAA 20<br>IA 10 | 41         | EA 19          | 19                | poor                                 | excellent                    | poor good                |

In Table 1

|      |                          |
|------|--------------------------|
| DAA  | Diacetone acrylamide     |
| LMA  | Lauryl methacrylate      |
| SA   | Stearyl acrylate         |
| SMA  | Stearyl methacrylate     |
| EHMA | Ethyl hexyl methacrylate |
| AA   | Acrylic acid             |
| MAA  | Methacrylic acid         |
| IA   | Itaconic acid            |
| MA   | Methyl acrylate          |
| MMA  | Methyl methacrylate      |
| EA   | Ethyl acrylate           |
| EMA  | Ethyl methacrylate       |
| BA   | Butyl acrylate           |
| BMA  | Butyl methacrylate       |

The results of the curl retention test carried out with respect to the hair lacquers prepared with the resin composition of Examples 1 - 3 are summarized in Table 2 in comparison with the results of the same test with respect to several hair lacquer products on the market.

Table 2

| Sample                | Time (hr.) | 0.5   | 1.0   | 1.5   | 2.0   | 2.5   | 3.0   | 10.0 |
|-----------------------|------------|-------|-------|-------|-------|-------|-------|------|
| Samples on the market |            |       |       |       |       |       |       |      |
| Sample A              | 92.0%      | 88.5% | 81.5% | 78.0% | 75.5% | 72.0% | 42.0% |      |
| Sample B              | 95.0%      | 93.0% | 88.0% | 85.0% | 81.5% | 77.0% | 58.0% |      |
| Sample C              | 91.0%      | 88.0% | 78.0% | 71.5% | 63.0% | 56.0  | 15.0% |      |
| Sample D              | 97.0%      | 92.5% | 90.5% | 88.5% | 84.0% | 73.0% | 20.0% |      |
| Sample from example 1 | 97.0%      | 96.0% | 93.0% | 91.5% | 89.0% | 85.5% | 70.0% |      |
| Sample from example 2 | 96.0%      | 91.0% | 88.0% | 82.5% | 78.0% | 77.0% | 66.0% |      |
| Sample from example 3 | 98.0%      | 94.5% | 92.5% | 90.0% | 87.5% | 83.0% | 67.5% |      |

Using these resin compositions, non-pressurized hair dressing preparations such as hair lotions and hair creams as well as skin cosmetics such as beauty packs and protective skin coatings were prepared. There was no difficulty in the preparation thereof as in preparation of the pressurized products.

Development of various products using the resin composition of this invention is under way.

What we claim is:

1. A resin composition useful in hair dressing preparations which comprises the resin-containing liquid obtained by refluxing the following copolymerizable monomeric ingredients at 78° - 90° C. in a water-soluble organic solvent:
  1. 5 - 89 percent by weight of a diacetone acrylamide,
  2. 5 - 40 percent by weight of at least one ester of an alkanol having four to 18 carbon atoms and an acid selected from a group consisting of acrylic acid and methacrylic acid,
  3. 6 - 35 percent by weight of at least one acid selected from a group consisting of acrylic acid, methacrylic acid and itaconic acid,
  4. 0 - 84 percent by weight of at least one ester of an alkanol having one to three carbon atoms and an acid selected from a group consisting of acrylic acid and methacrylic acid.
2. A resin composition as set forth in claim 1, wherein the copolymerizable monomeric mixture es-

sentially consists of (1) 10 - 60 percent by weight of diacetone acrylamide, (2) 10 - 30 percent by weight of at least one ester of an alkanol having four to 18 carbon atoms and an acid selected from a group consisting of acrylic acid and methacrylic acid, (3) 10 - 20 percent by weight of at least one acid selected from a group consisting of acrylic acid, methacrylic acid and itaconic acid, and (4) 20 - 70 percent by weight of at least one ester of an alkanol having one to three carbon atoms and an acid selected from a group consisting of acrylic acid and methacrylic acid.

3. A resin composition as set forth in claim 2, wherein the copolymerizable monomeric mixture essentially consists of (1) 20 - 30 percent by weight of diacetone acrylamide, (2) 15 - 30 percent by weight of an ester of an alkanol having four to 18 carbon atoms and at least one acid selected from a group consisting

of acrylic acid and methacrylic acid, (3) 10 - 20 percent by weight of at least one acid selected from a group consisting of acrylic acid, methacrylic acid and itaconic acid, and (4) 30 - 63 percent by weight of at least one ester of an alkanol having one to three carbon atoms and an acid selected from a group consisting of acrylic acid and methacrylic acid.

4. A resin composition as set forth in claim 1 which is neutralized with a basic substance.

5. A resin composition as set forth in claim 2 which is neutralized with a basic substance.

6. A resin composition as set forth in claim 3 which is neutralized with a basic substance.

7. A resin composition as set forth in claim 4 which is diluted with an water-miscible solvent.

8. A resin composition as set forth in claim 5, which is diluted with an water-miscible solvent.

9. A resin composition as set forth in claim 6, which is diluted with an water-miscible solvent.

10. A pressurized packaging system for hair dressing comprising the composition of claim 7 and a propellant.

11. A pressurized packaging system for hair dressing comprising the composition of claim 8 and a propellant.

12. A pressurized packaging system for hair dressing comprising the composition of claim 9 and a propellant.